

## UNITED STATES PATENT OFFICE

HERMANN FRITSCH, OF SWINEMUNDE, GERMANY, ASSIGNOR TO MESSRS. FOX, STOCKWELL & COMPANY, OF LONDON, ENGLAND

## BITUMINOUS ROAD SURFACE

No Drawing. Application filed October 30, 1929, Serial No. 403,666, and in Germany October 6, 1928.

This invention relates to a process for building bituminous street surfaces, poor of interstices and of an equal compactness from top to bottom, using stone material of graduated sizes, the bituminous treatment made in a cold process.

It is known, to bring stone material, aggregate and chips of uniform particle size to the foundation of a street, and to consolidate and to sprinkle it with tar or asphalt in the hot or cold process. For sealing the surface the top layer receives the known surface treatment.

These kinds of top layers (tar-grouted or bituminous grouted) have the drawback that owing to the missing of fine filling material numerous interstices remain in the top layer, and therefore the solidness and durability is greatly decreased, so that a large part of the binding substance sprinkled on the top layer runs through the interstices to the foundation, and the outer parts of the aggregate and chips are covered quite insufficiently by the binding substance, and in rainy weather these top layers, when treated in the hot process, remain for months, and when treated in the cold process, remain for weeks uncompleted and interrupt the traffic, till it is again dry weather. These top layers have also the disadvantage, that only the surface is sealed, that they lose of their compactness gradually to the bottom, therefore they have not sufficient compactness to resist the demands of the traffic for a longer period. This important drawback is not only caused by the insufficient filling of the binding substance, but also that the stone skeleton is not composed and consolidated according to the principle of a minimum of interstices, e. g., the mixture of the used stone material and the arrangement of the single chip and aggregate layers is not made to procure a minimum of interstices.

In the process according to this application, in which all the used materials in an efficient mixture and arrangement in layers are covered in the cold process on the building site with a binding substance, preferably with asphalt or tar emulsions or with efficiently prepared cold fluid tars or efficiently

prepared cold fluid asphalts and consolidated by one rolling down, these disadvantages will not appear, and therefore absolutely compact street surfaces with a minimum of interstices can be built also in unfavourable weather. Hitherto this could only be made in the hot process, and not even in a sufficient way and only in dry and warm weather, whereas the use of the tar macadam and tar concrete when the stone material must be covered in a hot condition with tar and brought to the building site in a cold condition and built in, has the large disadvantage, that the material during the transport and at the building site gets dirty and loses in its binding ability. The transport of the stone material and of the binding substance to a central point, where they are mixed, and the re-transport to the building site cause double loading and freight expenses, so that this process raises the price considerably. These top layers have also too many interstices, as the selection of the graduated sizes of the stone material, their mixture and arrangement in layers and the consolidation are not made according to the standard of this application, which is necessary to avoid the prejudicial interstices as much as possible. These road surfaces, constructed according to this application will never wave or corrugate or get slippery, in hot weather they will never soften or "bleed", contrary to the top layers, produced in the hot process, which show very often these disadvantages. This new kind of road surfaces can be made in three different methods, for instance:

## Example I. 6-10 cm. thick. Ingredients

|                                                                                                                                    | Millimeters | 90 |
|------------------------------------------------------------------------------------------------------------------------------------|-------------|----|
| Granite chips (aggregate) or furnace-cinder                                                                                        | 30-55       |    |
| Coarse granite chips or furnace-cinder                                                                                             | 15-30       |    |
| Medium granite chips                                                                                                               | 8-15        |    |
| Fine granite chips                                                                                                                 | 3-8         |    |
| Asphalt or tar emulsion (55-60% dry contents) or efficiently prepared cold fluid tars or efficiently prepared cold fluid asphalts. |             | 85 |

## Example II. 4-6 cm. thick. Ingredients

|                                                                                                                                    | Millimeters | 95  |
|------------------------------------------------------------------------------------------------------------------------------------|-------------|-----|
| Coarse granite chips or furnace-cinder                                                                                             | 15-30       |     |
| Medium granite chips                                                                                                               | 8-15        |     |
| Fine granite chips                                                                                                                 | 3-8         |     |
| Asphalt or tar emulsion (55-60% dry contents) or efficiently prepared cold fluid tars or efficiently prepared cold fluid asphalts. |             | 100 |

*Example III. 3-5 cm. thick. Ingredients*

|                                                                                                                                          | Millimeters |
|------------------------------------------------------------------------------------------------------------------------------------------|-------------|
| Coarse granite chips or furnace-cinder                                                                                                   | 15-30       |
| Medium granite chips                                                                                                                     | 8-10        |
| Smudge or sand                                                                                                                           | 0, 2-0, 6   |
| Sand                                                                                                                                     | 0-0, 2      |
| Asphalt or tar emulsion (55-60% dry contents) or<br>efficiently prepared cold fluid tars or efficiently<br>prepared cold fluid asphalts. | 5           |

The road surfaces are made in two different layers as follows:

- On the old or new macadam or paving surface, which must at first be levelled down and profiled, the coarse binding layer is brought up, after the used stone is well mixed and impregnated with one of the above mentioned cold binding substances, either by hand on a mixing board, or by machine. A second fine filling layer is at once and according to the profile put on this lower binding layer, impregnated as the binding layer. When using emulsions, they are broken after the mixture with the stone material and the impregnation, i. e. the decay has taken place, the precipitated particles of tar or asphalt have caused a close lutation of the stone and cinder ingredients. When using cold fluid tars or cold fluid bitumina the mixing and impregnation process also takes place at once during the mixing. The mineral layers, impregnated in this way, are still ductile and can be moulded, as the bitumina or tars do not congeal at once, but are flexible. Now the top layer is consolidated with a street roller of medium weight. As the mixture of the graduated sizes of the stones and the arrangement of the layers has been chosen to attain a minimum of interstices, the fine filling layer is pressed into the lower binding layer by the consolidation, so that parts of the top layer penetrate to the foundation and remove nearly completely all interstices. Preferably the accordingly mixed and arranged impregnated stone material is pressed into each other through a single rolling in the above mentioned way. If first the lower, and then the top layer would be rolled, as done hitherto, the lower layer would be already hard and luted, so that the fine stone material of the top layer could not penetrate into the lower and fill the still existing interstices.
- Hereafter or after about a fortnight the top layer, which is consolidated in the meantime, receives a slight surface treatment with impregnated fine chips or sand to seal the small pores of the surface, should there be any.
- What I claim is:
1. The process for the construction and paving of roads which comprises applying to a suitable foundation a layer consisting in a mixture of relatively coarse and relatively finer aggregate coated with bituminous composition fluid in the cold and superimposing thereon a plurality of layers of mixed aggregate coated with bituminous composition fluid in the cold, the aggregate of each of said
- 60
- 65
- 50
- 55
- 60
- 65

layers having a greater average degree of subdivision than the layer on which it is superimposed and each of the several layers consisting of particles of different sizes in proportions adapted to yield a mixture having a minimum of voids and thereafter rolling the whole.

2. The process for the construction and paving of roads which comprises applying to a suitable foundation a layer consisting in a mixture of relatively coarse and relatively finer aggregate coated with bituminous emulsion and superimposing thereon a plurality of layers of mixed aggregate coated with bituminous emulsion fluid in the cold, the aggregate of each of said layers having a greater average degree of subdivision than the layer on which it is superimposed and each of the several layers consisting of particles of different sizes in proportions adapted to yield a mixture having a minimum of voids and thereafter rolling the whole.

3. The process for the construction and paving of roads which comprises applying to a suitable foundation a layer consisting in a mixture of relatively coarse and relatively finer aggregate coated with bituminous composition fluid in the cold and superimposing thereon a plurality of layers of mixed aggregate freshly coated at the place of use with bituminous composition fluid in the cold, the aggregate of each of said layers having a greater average degree of subdivision than the layer on which it is superimposed and each of the several layers consisting of particles of different sizes in proportions adapted to yield a mixture having a minimum of voids and thereafter rolling the whole.

4. The process for the construction and paving of roads which comprises applying to a suitable foundation a layer consisting in a mixture of relatively coarse and relatively finer aggregate coated with bituminous emulsion and superimposing thereon a plurality of layers of mixed aggregate freshly coated at the place of use with bituminous emulsion, the aggregate of each of said layers having a greater average degree of subdivision than the layer on which it is superimposed and each of the several layers consisting of particles of different sizes in proportions adapted to yield a mixture having a minimum of voids and thereafter rolling the whole.

In testimony whereof I have signed my name to this specification.

HERMANN FRITSCH.